

[54] **SULFURIZED MONO-ESTERS OF TALL OIL FATTY ACIDS AND PRIMARY OXO ALCOHOLS**[75] Inventors: **Norman Arthur Carlson, Wilmington; Bruce Hollis Garth, Newark, both of Del.**[73] Assignee: **E. I. du Pont de Nemours and Company, Wilmington, Del.**[22] Filed: **Feb. 23, 1972**[21] Appl. No.: **228,749**[52] U.S. Cl. .... **260/97.5, 252/48.6, 260/399, 260/468.5**[51] Int. Cl. .... **C09f 1/00**[58] Field of Search..... **260/97.5, 468.5, 399; 252/48.6**[56] **References Cited**

## UNITED STATES PATENTS

2,179,065 11/1939 Smith ..... 260/399

|           |         |               |          |
|-----------|---------|---------------|----------|
| 2,179,066 | 11/1939 | Smith.....    | 260/399  |
| 2,644,810 | 7/1953  | Beretrás..... | 260/97.5 |
| 2,683,119 | 7/1954  | Smith.....    | 252/48.6 |
| 2,815,368 | 12/1957 | Matuszak..... | 252/48.6 |
| 2,820,054 | 1/1958  | Matuszak..... | 252/48.6 |
| 2,884,379 | 4/1959  | Rudel.....    | 252/48.6 |
| 2,891,084 | 6/1959  | Alm .....     | 260/97.5 |

*Primary Examiner*—Donald E. Czaja*Assistant Examiner*—Eugene C. Rzucidlov*Attorney, Agent, or Firm*—Nicholas J. Masington, Jr.; James A. Costello[57] **ABSTRACT**

Sulfurized mono-esters of tall oil fatty acids and branched chain primary alcohols of six to 20 carbon atoms.

**5 Claims, No Drawings**

## SULFURIZED MONO-ESTERS OF TALL OIL FATTY ACIDS AND PRIMARY OXO ALCOHOLS

### BACKGROUND OF THE INVENTION

#### 1. Field of the Invention

This invention relates to sulfurized mono-esters. More particularly this invention relates to sulfurized tall oil fatty acid esters of  $C_6$  to  $C_{20}$  branched chain saturated primary alcohols, which esters are effective extreme pressure additives.

#### 2. Description of the Prior Art

Modern lubricants are complex mixtures of base lubricant fluids and additives. A lubricant additive is generally defined as a material which imparts a new and desirable property which is not possessed by the base lubricant fluid or which enhances certain desirable characteristics of such fluid. Additives are used for such purposes as to decrease oxidative and thermal degradation of the oil, reduce formation of deposits, reduce rust and corrosion, reduce friction and wear and to prevent destructive metal-to-metal contacts.

With the advent of high performance automobiles, the importance and need for lubricant additives which prevent destructive metal-to-metal contact has greatly increased. As is well-known in the art, plain mineral oils provide good lubrication between moving metal parts as long as a film of oil is maintained between them. However, when pressures or rubbing speed between the moving metal surfaces are such that the film of oil is squeezed or wiped out, destructive metal-to-metal contact occurs over a significant portion of the contacting metal surfaces. Adverse consequences of such metal-to-metal contact, often referred to as boundary lubrication, include welding, scoring, scuffing and in some cases, deformation or destruction of the lubricated components. Situations wherein boundary lubrication might occur include operating hypoid gears, automatic transmissions, limited slip differentials, metal cutting and metal drawing operations and the like. Extreme pressure (EP) additives are employed in the lubricants to prevent the above-described destructive metal-to-metal contact. It is believed that EP additives function by reacting with metal surfaces under boundary lubricating conditions to form an adherent film of metal salts. This film then acts as a solid lubricant when conditions of metal-to-metal contact occur. A necessary property of effective EP additives is that the formation of the film of metal salts takes place only at elevated temperatures which develop locally between the moving metal parts under conditions of boundary lubrication. If the formation of the metal salt film takes place under conditions other than that described above, for example at lower temperatures, excessive corrosion of the metal parts can take place whereas if the additive is too stable to react with the metal surface under boundary lubrication conditions, the additive will be ineffective as an extreme pressure additive.

The majority of art-known, effective EP additives are organic compounds which contain chemically bound sulfur, phosphorous, or chlorine or which contain functional groups such as carboxyl. Because of the lower cost, availability, and effectiveness, sulfurized sperm oil has been used extensively as an EP additive. Sperm oil is obtained from the head cavity and blubber of sperm whales, refined and sulfurized.

The well-known sulfurized sperm oil is principally sulfurized fatty acid mono-esters of relatively high molecular weight monohydric alcohols. Typically, the fatty acids are present in these whale oils as mono-esters of high molecular weight alcohols. The alcohol portions of the whale oil monoesters are principally monohydric alcohols which are of corresponding chain length as the fatty acids and with about the same degree of unsaturation.

10 Sulfurized sperm oil of commerce is produced by treating refined sperm oil with sulfur in the temperature range of 300° to 385°F. Crude sperm oil contains varying amounts of spermaceti and other solid waxes. In refining the crude sperm oils, these waxes are removed by refrigeration and pressing. In U.S. Pat. No. 2,179,066 a process of sulfurizing sperm oil is disclosed wherein the sperm oil is reacted with suitable amounts of sulfur at temperatures of about 300° to 385°F., the reaction being continued until sulfur is combined in the form of neutral sulfur compounds.

15 Recently, however, there has been increasing concern over the rapid decrease in the world's whale population, and consequently importation of whale oil into the United States has been banned. It has thus become necessary to provide a substitute for sulfurized sperm oil.

20 It is known in the art to sulfurize mono-esters generally to produce sulfurized esters useful as lubricant additives. For example, Smith in U.S. Pat. No. 2,179,065 discloses sulfurized esters prepared by sulfurizing compounds of the formula



35 wherein R and  $R_1$  are straight chain aliphatic groups and at least one of R and  $R_1$  being olefinic group.

40 Beretvas in U.S. Pat. No. 2,644,810 discloses a process for sulfurizing esters by treating mono-esters with sulfur chloride in the presence of water. The disclosed mono-esters suitable for sulfurization are unsaturated mono-esters of aliphatic acids having the general formula



50 wherein R is a hydrocarbon group of straight chain aliphatic group or an unsaturated cycloaliphatic group,  $R_1$  is a straight chain aliphatic hydrocarbon group and X is oxygen or sulfur.

55 Generally, however, commercially available products suggested as replacements for sulfurized sperm oil have been deficient in at least one or more of the properties necessary for a useful EP additive, e.g. lack of solubility in base lubricant oil, lack of stability of solutions in base oil, insufficiently high flash point or in undesirably high pour point.

60 Sulfurized esters have now been discovered which are useful as extreme pressure additives, are inexpensive to produce, and have superior characteristics of good and stable solubility in lubricant bases, lower viscosities, higher flash points, and lower pour points. Those and the other objectives of the invention will be apparent from the discussion which follows.

## SUMMARY OF THE INVENTION

This invention is directed to a composition comprising sulfurized tall oil fatty acid esters of  $C_6$  to  $C_{20}$  branched chain saturated primary alcohols.

## DESCRIPTION OF THE INVENTION

It has now been discovered that when mono-esters of tall oil fatty acids and branched chain saturated primary alcohols of six to 20 carbon atoms are sulfurized, products suitable as lubricant additives are obtained. The sulfurized products are effective as extreme pressure additives and as anti-wear additives.

Tall oil fatty acids useful in preparing the sulfurized mono-esters of the present invention are obtained from the spent black liquor of pulping processes. The black liquor is concentrated until the sodium salts of the various acids separate out and are skimmed off. The acids are obtained by acidification and then purified. Since tall oil fatty acids are by-products of extensive pulping operations, such acids are readily and economically available. Typically tall oil fatty acids contain mixtures of fatty acids having from about 14 carbon atoms to about 22 carbon atoms with oleic acid (30-50 percent) and linoleic acid (35-42 percent) comprising the major portion of such acid mixtures. Tall oil fatty acids also contain small amounts of saturated acid, e.g., about 1-10 percent as well as trace amounts of tri-unsaturated acids. Tall oil fatty acids comprising from about 75 to about 99% of unsaturated monocarboxylic acids having from 16 to 18 carbon atoms are particularly useful in the preparation of the sulfurized esters of the invention, a mixture of oleic and linoleic acids being most useful. Preferred tall oil fatty acids will comprise from about 40 percent to about 50 percent by weight of oleic acid and from about 35 to about 50 percent of linoleic acid based on the total weight of the tall oil fatty acid. More preferred tall oil fatty acids comprise from about 45 to about 50 percent by weight of oleic acid and from about 50 to about 45 percent by weight of linoleic acid. While a single component of tall oil fatty acid e.g., all oleic acid may be used to prepare the sulfurized ester, the tall oil fatty acid containing the aforementioned mixture of acids is preferred since sulfurized esters prepared therefrom provide better (lower) pour point, and are available more economically.

The alcohols useful in preparing the products of the invention are branched chain saturated primary alcohols of six to 20 carbon atoms. Because of their availability and low cost, the preferred branched chain saturated aliphatic primary alcohols are oxo alcohols having from about six to about 20 carbon atoms. The oxo alcohols are produced by the art known process of subjecting an olefin, containing one less carbon than the desired alcohol, to a carbonylation reaction at pressures of from about 1,000 to 3,000 psi. and a temperature of from about 300° to 400°F. with carbon monoxide and hydrogen in the presence of carbonylation catalyst such as cobalt carbonyl. The aldehydes which are the reaction products of this carbonylation reaction are then hydrogenated to form the desired alcohols.

Oxo hexyl alcohol, for example, is prepared by carbonylation and hydrogenation of an olefin which is prepared by the condensation of propylene and ethylene. The oxo hexyl alcohols contain 3 methyl- and 4 methyl-pentanols as principal branched chain saturated primary alcohols. The oxo alcohol of 8 carbon atoms is

prepared by carbonylation and hydrogenation of propylene-butylene condensation product. The  $C_8$  oxo alcohols thus obtained are primary alcohols with dimethylhexanols being the major components thereof. Similarly,  $C_{10}$  oxo alcohols may be prepared from propylene trimer,  $C_{13}$  oxo alcohol from propylene tetramer,  $C_{16}$  oxo alcohols from propylene pentamers. In general, olefins containing one less carbon atom than the desired alcohol can be prepared by the proper combination of readily available olefins, for example, combining 5 parts of propylene with 1 part of butylene to form olefins containing 19 carbon atoms which can then be carbonylated and hydrogenated to provide oxo alcohol of 20 carbon atoms. While any one of the alcohols present in the oxo alcohols of six to 20 carbon atoms may be used alone to provide mono-ester of tall oil fatty acids which are then sulfurized, it is preferable to use oxo alcohols which are mixtures because of their availability and lower costs. The preferred oxo alcohol for the preparation of the products of the invention is oxo decyl alcohol.

The mono-esters of useful tall oil fatty acids and branched chain primary alcohols of six to 20 carbon atoms may be prepared by any art known esterification procedure. Esterification catalysts such as hydrochloric acid, sulfuric acid, ethanesulfonic acid, toluenesulfonic acid may be used. When the esterification process is carried out in steel vessels, mono-alkyl and dialkyl esters of ortho phosphoric acid may be used advantageously since the corrosion of steel vessels is minimized by their use.

The  $C_6$ - $C_{20}$  oxo alcohol mono-esters of tall oil fatty acids can be sulfurized by art-known methods. For example, a mixture of the mono-ester and sulfur can be heated to about 160°C. to 180°C. for about 7 hours. The sulfur may be any relatively good grade of sulfur such as flowers of sulfur or screened sulfur. Preferably the sulfur is in a subdivided state for ease of reaction and for better reaction control. The amount of sulfur used and the temperature employed will depend upon the particular sulfurized ester desired and can be readily determined by one skilled in the art.

Generally in the trade, sulfurized products are used as extreme pressure additives in three fields of applications: (1) "Mild" or low activity as in worm gear oils, manual gear box oils, motor oils, steam turbine oils, hydraulic oils and the like; (2) "moderate" or intermediate as in hypoid gear oils and industrial gear oils; and (3) "high" activity as in cutting oils, metal drawing compounds, metal forming oils and in some hypoid gear oils. For mild or moderate activity, the sulfurized compounds usually contain about 10 percent or less of combined sulfur whereas for high activity the combined sulfur content is greater than about 10 percent, usually around 15-16%.

For the preparation of sulfurized esters of this invention of  $C_6$  to  $C_{20}$  oxo alcohols and tall oil fatty acids containing about 10 percent combined sulfur, heating of a mixture of the mono-ester with a slight excess (10 percent) of sulfur at about 180°C. for about 7 to 12 hours will produce sulfurized ester containing about 10 percent combined sulfur. During the reaction a very small amount of hydrogen sulfide is evolved.

The sulfurized compositions of this invention normally contain from about 5 percent by weight to about 16 percent by weight of sulfur based on the weight of the sulfurized composition. For the preparation of sul-

furized esters of this invention containing more than 10% combined sulfur, the reaction is preferably carried out at around 160°C. since at 180°C. greater amounts of dehydrogenation reaction with accompanying great formation of hydrogen sulfide takes place.

As has been stated previously and will be shown in more detail in the examples, the compositions of this invention, i.e., the sulfurized C<sub>6</sub>–C<sub>20</sub> oxo alcohol mono-esters of tall oil fatty acids, are effective extreme pressure additives for lubricants. The compositions of the invention have additional desirable properties such as (1) being highly soluble and stable in solvent refined neutral oil, (2) low viscosity, (3) high flash point, (4) very low pour point, and (5) compatibility with lead naphthenate.

Any additive for lubricant should, of course, have good solubility in the base oil to which it is added and the solutions thus prepared should be stable over extended periods of time. Since sulfurized additives are often used in concentrations of up to 20 percent, by weight of the formulated lubricant compositions, it is desirable that these sulfurized additives have high solubility. The sulfurized compositions of this invention are soluble to at least 50 percent by weight in solvent neutral oils and the resultant solutions are stable for extended periods of time.

For ease and safety in blending with lubricant base, it is often desirable that the sulfurized additives have low viscosity, high flash point and low pour point. A preferred composition of this invention, i.e., the oxo decyl ester of tall oil fatty acids sulfurized to contain about 10 percent combined sulfur has a viscosity of 61 SUS at 210°F., flash point of 465°F. and a pour point of -40°F. By way of comparison, a typical sulfurized sperm oil containing about 10 percent combined sulfur has a viscosity of about 200 to 250 SUS at 210°F., a flash point of about 425°F. and a pour point of 45° to 55°F.

The compositions of this invention may be poured or pumped much more readily than sulfurized sperm oil for blending purposes because of the lower viscosity and considerably lower pour point. Since the sulfurized ester may comprise up to about 20 percent by weight of the lubricant composition, it is clear that sulfurized esters of low pour point are highly desirable, not only in that they facilitate formulation of the lubricant compositions, but also in that they do not increase the pour

point of the formulated lubricant. Further, it is clear to those skilled in the art that high pour point lubricants are not desirable, since they may provide inadequate lubrication at low temperatures.

In certain applications involving high speed and high torque services, lubricants containing lead soaps such as lead naphthenates in addition to the sulfurized additives are often used. It is highly desirable therefore, that the sulfurized additives provide extreme pressure characteristics which can be utilized in conjunction with the extreme pressure characteristics of the lead soaps. It is also highly important that the sulfurized additives be compatible (i.e., do not form precipitates) when mixed with lead soaps. The compositions of the present invention provide extreme pressure characteristics which complement the extreme pressure characteristics of lead naphthenate and the mixture of the sulfurized esters of this invention with lead naphthenate is compatible. As shown in Example 16, practically all of sulfurized products, now offered commercially as substitutes for sulfurized sperm oil are not compatible with lead naphthenate.

The lubricant base to which the compositions of the present invention may be added comprise any petroleum lubricating oil fraction such as a neutral or bright stock oil of any suitable viscosity. The amount of the sulfurized ester used and the particular viscosity of the lubricant base used will depend upon the particular use intended for the lubricant composition to be prepared. The sulfurized esters of the invention may be used together with the conventional lubricant additives such as antioxidants, anti-wear agents, viscosity index improvers, pour point depressants, and the like.

## EXAMPLES

The following examples are intended to be merely illustrative of the invention and not in limitation thereof. Unless otherwise indicated, all quantities are by weight.

### EXAMPLE 1

This example describes the preparation of sulfurized tall oil fatty acid esters of oxy decyl alcohol. Tall oil fatty acids used were "Acintol" Tall Oil Fatty Acids sold by Arizona Chemical Company. The "Acintol" tall oil fatty acids are available in several grades; the compositions and designations as supplied by the manufacturer are given in the following table.

Table 1

| Acids (By gas chromatograph)            | TALL OIL FATTY ACIDS<br>Tall Oil Fatty Acid Designation |      |                 |      |      |
|-----------------------------------------|---------------------------------------------------------|------|-----------------|------|------|
|                                         | DGLR                                                    | FA-1 | FA-1<br>Special | FA-2 | FA-3 |
| Lower Boiling Acids, %                  | 0.1                                                     | —    | —               | —    | —    |
| Palmitic Acid, %                        | 5.3                                                     | 2.3  | 1.9             | 0.1  | 0.1  |
| Palmitoleic Acid, %                     | 2.1                                                     | 0.6  | 1.2             | 0.2  | 0.1  |
| Unknown Acid, %                         | 0.3                                                     | 0.3  | 0.1             | 0.1  | 0.1  |
| Stearic Acid, %                         | 2.1                                                     | 2.3  | 2.2             | 2.5  | 2.6  |
| Oleic Acid                              | 39.3                                                    | 41.0 | 43.0            | 49.5 | 48.0 |
| Unknown Acid, %                         | 1.6                                                     | 1.2  | 1.7             | 1.6  | 2.0  |
| Linoleic Acid (cis-9,cis-12)%,          | 29.4                                                    | 32.8 | 32.2            | 35.7 | 38.1 |
| Unknown Acid, %                         | 2.3                                                     | 2.5  | 2.5             | 3.1  | 2.7  |
| Unknown Acid, %                         | 0.9                                                     | 0.6  | 0.9             | 0.4  | 0.2  |
| Linoleic Acid<br>(cis-9, trans-11), %   | 4.3                                                     | 3.8  | 4.4             | 2.6  | 2.4  |
| Eicosanoic Acid, %                      | 1.7                                                     | 1.9  | 1.8             | 1.4  | 1.2  |
| Linoleic Acid<br>(trans-9, trans-11), % | 4.4                                                     | 4.8  | 4.3             | 1.2  | 1.4  |
| Eicosadienoic Acid, %                   | 3.2                                                     | 2.1  | 1.1             | 0.5  | 0.5  |
| Eicosatrienoic Acid, %                  | 2.6                                                     | 2.9  | 1.9             | 0.4  | 0.6  |
| Behenic Acid, %                         | 0.4                                                     | 0.9  | 0.8             | 0.7  | —    |
| Higher Boiling Acids, %                 | —                                                       | —    | —               | —    | —    |

The oxo decyl alcohol was purchased from Enjay.

### ESTERIFICATION

"Acintol" FA-3 (4725 g.), oxo decyl alcohol (2861 g.) and tridecyl acid phosphates (22 g.) were heated in a reaction vessel at 180°C. under nitrogen sweep. After about 13 hours, evolution of water ceased and the infra-red analysis of the reaction mixture indicated completion of the esterification reaction (absence of absorbance due to carboxylic acid group). The reaction product mixture was then stripped for five hours by passing nitrogen into the charge at 180°C. under a vacuum of about 20 to 50 mm. Hg pressure to remove unreacted alcohol. The yield of resultant "Acintol" FA-3 oxo decyl ester was 7125 g. (theory 7128 g.).

### SULFURIZATION (10% SULFUR)

A mixture of 2816 g. of the "Acintol" FA-3 oxo decyl ester prepared above and 313 g. of screened sulfur was heated at 180°C. under nitrogen sweep for 7 hours, then at 180°C. and a vacuum of 20 mm. Hg. pressure for 1 hour and finally at 180°C. with nitrogen passage through the charge under a vacuum of 20 to 50 mm Hg. pressure for three hours. The exit gases were passed through a caustic scrubber containing 20 percent aqueous sodium hydroxide to trap a small amount of hydrogen sulfide evolved. The yield of sulfurized dark brown clear fluid was 3106 g. Analysis for sulfur showed combined sulfur content of 9.9 percent. The sulfurized ester had a viscosity of 61 SUS at 210°F., a saponification number of 145, an acid number of 2.1, flash point (Cleveland Open Cup) of 465°F. and a pour point of -40°F. The sulfurized ester exhibited excellent solubility in neutral solvent oils (100 SUS at 100°F) of both naphthenic and paraffinic origins, being soluble to greater than 50 percent by weight at room temperature. A 10 percent solution of the sulfurized ester in the above neutral oil stored over one month remained clear with no evidence of haze or precipitate.

Sulfurized esters containing less than about 12 percent combined sulfur can be prepared by essentially the general procedure described above, by using the appropriate amount of sulfur. Generally, the amount of sulfur used is about 10 percent in excess of the desired sulfur content of the final sulfurized product; however, anyone skilled in the art can readily determine the exact proportion of sulfur to ester to be used to obtain the de-

sired sulfur content in the sulfurized ester by relatively few experiments. When sulfurized esters containing more than about 12 percent sulfur are desired, it is preferable to carry out the sulfurization reaction at about 160°C. instead of at 180°C. in order to reduce the amount of dehydrogenation reaction.

### EXAMPLES 2-14

Using the general procedures described in Example 1, additional sulfurized tall oil fatty esters were prepared. The useful additive property date of these esters including copper strip corrosion pour point, and solubility are set out in Table II below. Both the copper strip corrosion and the solubility tests were carried out with a 10 percent by volume solution of the sulfurized ester in 100 SUS/100°F. solvent-refined neutral oil (Sun SSR-110, Sun Oil Co.). Copper strip corrosion tests were carried out according to ASTM D-130. In the ASTM D-130 test, the results are indicated by classification by numbers of from 1 to 4 wherein 1 indicates very slight tarnish and 4 indicates extensive corrosion. The solubility test was carried out by keeping the 10 volume percent solution of the sulfurized ester in the neutral oil at room temperature and observing for the formation of haze or precipitate over a period of time. If the solution remained clear over a period of one month, the solubility is designated as satisfactory. The pour points of sulfurized esters were determined by ASTM D-97 method. The lowest temperature (°F.) at which the sulfurized ester was observed to flow when cooled and examined under prescribed conditions is recorded as pour point.

These examples also illustrate that the compositions of the present invention show good copper strip corrosion resistance, good solubility characteristics and unexpectedly low pour point characteristics. As mentioned earlier, a typical sulfurized sperm oil has pour point in the range of 45° to 55°F. The copper strip corrosion values of 4 as shown for examples 7, 8 and 9 are expected and desirable because sulfurized products containing greater than about 12 percent sulfur are generally used in applications requiring high extreme pressure activity, e.g., in cutting oils. Sulfur compounds having a high degree of activity are known in the industry as "corrosive sulfur" additives and thus require the degree of activity in corrosion tests indicated by the composition of examples 7, 8 and 9.

Table II

| Example | Acid           | Alcohol         | SULFURIZED TALL OIL FATTY ACID ESTERS |                | Copper Strip Corrosion Test | Solubility Test |
|---------|----------------|-----------------|---------------------------------------|----------------|-----------------------------|-----------------|
|         |                |                 | % Combined Sulfur                     | Pour Point °F. |                             |                 |
| 2       | "Acintol" FA-3 | Hexyl (oxo)     | 10.2                                  | -15            | 1                           | Satis.          |
| 3       | "Acintol" FA-3 | Decyl (oxo)     | 6.0                                   | -20            | 1                           | do.             |
| 4       | "Acintol" FA-3 | Decyl (oxo)     | 9.3                                   | -40            | 1                           | do.             |
| 5       | "Acintol" FA-1 | Decyl (oxo)     | 9.8                                   | -20            | 1                           | do.             |
| 6       | "Acintol" FA-3 | Decyl (oxo)     | 12.0                                  | -20            | 1                           | do.             |
| 7       | "Acintol" FA-3 | Decyl (oxo)     | 13.6                                  | -20            | 4                           | do.             |
| 8       | "Acintol" FA-3 | Decyl (oxo)     | 15.7                                  | -40            | 4                           | do.             |
| 9       | "Acintol" FA-3 | Decyl (oxo)     | 16.0                                  | -20            | 4                           | do.             |
| 10      | Oleic          | Decyl (oxo)     | 9.1                                   | -20            | 2                           | do.             |
| 11      | "Acintol" FA-3 | n-Decyl         | 9.9                                   | +10            | 1                           | do.             |
| 12      | "Acintol" FA-3 | Tridecyl (oxo)  | 9.7                                   | -40            | 1                           | do.             |
| 13      | "Acintol" FA-3 | n-Hexadecyl     | 9.8                                   | +80            | 1                           | do.             |
| 14      | "Acintol" FA-3 | Hexadecyl (oxo) | 9.0                                   | -45            | 1                           | do.             |

## EXAMPLE 15

This example illustrates the extreme pressure additive activity of the sulfurized esters of this invention and in addition, compares the characteristics of the compositions of this invention with some of the art-known products utilized in the trade as substitutes for sulfurized sperm oil. The extreme pressure properties were determined by Federal Test Method Standard (FTMS) 6503. The test consists of pressing a rotating steel ball against a triangle of specimen-lubricated stationary steel balls. The test apparatus used was a Shell Four Ball Extreme Pressure Tester. In carrying out the test, force was applied to the balls until welding occurred. Welding was detected by a sharp movement of the indicating pen signifying momentary locking of the four balls. All tests were carried out with 10 percent by volume of sulfurized products in 100 SUS/100°F. neutral oil. The solubility tests, copper strip corrosion tests and pour point determination were carried out as described in the previous examples. Flash point (Cleveland Open Cup) determinations were carried out according to ASTM D-92. The art-known commercially available products used in this example for comparison with the products of the invention are designated A, B and C, and since these products are offered with different levels of sulfur, further designations as A-1, A-2, etc. is used. The chemical compositions of these commercially available sulfurized products were not determined. However, it is known that these products have been offered as commercial substitutes for sulfurized sperm oil. Also, for purposes of comparison, the data for a typical sulfurized sperm oil are also included. The comparative data are set out in Table III below.

Table III clearly shows that the sulfurized esters of the present invention possess extreme pressure lubricating properties superior to the commercial products A, B and C and in addition have highly desirable characteristics of high flash points and low pour points. It should also be noted that the sulfurized esters of this invention have higher flash point and lower pour point than sulfurized sperm oil.

## Example 16

Lead soaps, such as lead naphthenate, are often used with sulfurized products to provide lubricants which

have good protection against scoring of metal surfaces in high speed and high torque services. This example shows that the sulfurized esters of this invention may be successfully used in conjunction with lead naphthenate and that they are compatible with lead naphthenate. Table IV shows the four ball weld point data of 10 percent by volume of (a) the sulfurized ester of the Example, (b) a 10 percent solution of lead naphthenate and (c) of the combination of the sulfurized ester with lead naphthenate. It is seen from the Table IV that the extreme pressure activity of the sulfurized esters of Example 1 complements the extreme pressure activity of lead naphthenate when used together. The Four Ball Extreme Pressure tests were carried out as described in Example 15 using solvent neutral oil (100 SUS/100°F.) as the base oil.

Table IV

| SULFURIZED ESTER - LEAD NAPHTHENATE COMBINATION |                                                 | Four Ball<br>Weld Point(Kg.) |
|-------------------------------------------------|-------------------------------------------------|------------------------------|
| (a)                                             | 10 Vol. % Example 1                             | 178                          |
| (b)                                             | 10% Lead Naphthenate                            | 224                          |
| (c)                                             | 10% Vol. % Example plus<br>10% Lead Naphthenate | 400                          |

The data of Table V show that the sulfurized esters of the present invention are compatible with lead naphthenates. The compatibility test was carried out by adding lead naphthenate (3 percent) and various sulfurized products (4 percent) to a base lubricant stock prepared by mixing one part of 350 SUS/100°F. neutral oil and three parts of bright stock. The mixtures were stored at 150°F. and is inspected daily for deposit formation. If no deposit formation took place during the first week, the composition was considered to pass the compatibility test. If the tested composition failed the test, the number of days to failure is indicated in Table V. Compositions B-1 and 2, C-1 and 2 and D-G represent commercially available sulfurized products offered as sulfurized sperm oil substitutes.

Table III

| Composition                                             | % Sulfur | Initial       | COMPARISON OF SULFURIZED PRODUCTS |              | Pour Point % | Flash Point % | Copper Strip Corrosion | Weld Test Kg. Load |
|---------------------------------------------------------|----------|---------------|-----------------------------------|--------------|--------------|---------------|------------------------|--------------------|
|                                                         |          |               | Solubility Test (1)<br>2 Weeks    | 1 Month      |              |               |                        |                    |
| A-1                                                     | 10-11    | *Satisfactory | ppt.                              | —            | + 50         | 410           | 1                      | —                  |
| A-2                                                     | 14-15    | Haze          | ppt.                              | —            | + 60         | 410           | 4                      | —                  |
| B-1                                                     | 10       | Satisfactory  | Satisfactory                      | Satisfactory | + 40         | 410           | 1                      | 158                |
| B-2                                                     | 11.5     | do.           | do.                               | ppt.         | + 40         | 410           | 1                      | 178                |
| B-3                                                     | 17       | do.           | do.                               | Satisfactory | + 45         | 405           | 4                      | 224                |
| C-1                                                     | 10       | do.           | do.                               | ppt.         | + 65         | 420           | 1                      | 126                |
| C-2                                                     | 12       | do.           | ppt.                              | —            | —            | —             | —                      | 141                |
| Sulfurized Sperm Oil Invention Composition of Example 1 | 11.5     | do.           | Satisfactory                      | Satisfactory | + 55         | 425           | 1                      | 200                |
| Invention Composition of Example 9                      | 9.9      | do.           | do.                               | do.          | + 40         | 465           | 1                      | 178                |
| Invention Composition of Example 9                      | 16.0     | do.           | do.                               | do.          | + 20         | 465           | 4                      | 224                |

\* Satisfactory indicates clear solution; ppt - precipitate.

Table V

| Composition                        | %S   | LEAD NAPHTHENATE COMPATIBILITY |               | Test No. Days |
|------------------------------------|------|--------------------------------|---------------|---------------|
|                                    |      | Pass or Fail                   | Compatibility |               |
| Sulfurized Sperm Oil               | 10   | X                              |               | —             |
| Invention Composition of Example 1 | 9.9  | X                              |               | —             |
| Commercial Product B-1             | 10   |                                | X             | 5             |
| Commercial Product B-2             | 11.5 |                                | X             | 1             |
| Commercial Product C-1             | 10   |                                | X             | 1             |
| Commercial Product C-2             | 12   |                                | X             | 1             |
| Commercial Product D               | 11   |                                | X             | 5             |
| Commercial Product E               | 10   |                                | X             | 5             |
| Commercial Product F               | 10   |                                | X             | 5             |
| Commercial Product G               | 11   |                                | X             | 1             |

The foregoing detailed description has been given for clarity of understanding only and no unnecessary limitations are to be understood therefrom. The invention is not limited to exact details shown and described for obvious modifications will occur to one skilled in the art.

The embodiments of the invention in which an exclusive property or privilege is claimed are defined as follows:

1. A composition comprising sulfurized tall oil fatty acid mono-esters of C<sub>6</sub> to C<sub>20</sub> branched chain saturated primary oxo alcohols wherein the amount of sulfur present is from about 5 to 16 percent based on total weight of the composition.

2. A composition according to claim 1 wherein the tall oil fatty acid of the ester comprises from about 75 to about 99 percent by weight of unsaturated monocarboxylic acids having from 16 to 18 carbon atoms based on the total weight of the fatty acid.

3. A composition according to claim 1 wherein the tall oil fatty acid of the ester comprises from about 40 to about 50 percent by weight of oleic acid and from about 35 percent to about 50 percent by weight of linoleic acid based on the total weight of the fatty acid.

4. A composition according to claim 3 wherein the tall oil fatty acid of the ester comprises from about 45 to about 50 percent by weight of oleic acid and from about 40 percent to about 45 percent by weight of linoleic acid based on the total weight of the fatty acid.

5. A composition according to claim 1 wherein the oxo alcohol is oxo decyl alcohol.

\* \* \* \* \*

25

30

35

40

45

50

55

60

65